

## UNITED STATES PATENT OFFICE

2,263,239

## MOTOR FUEL

George H. Freyermuth, Scarsdale, and Anthony E. Robertson, New York, N. Y., assignors to Standard Oil Development Company, a corporation of Delaware

No Drawing. Application August 24, 1939,  
Serial No. 291,684

2 Claims. (Cl. 44—9)

The present invention relates to improved motor fuels and method of preparing same and it relates more particularly to the preparation of motor fuels having high anti-detonation properties.

It has been known for some time that the class of chemical compounds known as "diolefines" have high anti-knock value when blended in gasoline for use as motor fuel. However, especially when present along with other highly unsaturated compounds formed during the vapor phase cracking of heavy hydrocarbons to make gasoline, they have the serious disadvantage of tending to induce the formation of large amounts of gum owing to the peculiar susceptibility of the chemical structure of the various highly unsaturated hydrocarbons to oxidation and polymerization or condensation and/or other chemical reactions involved in the formation of gum. The exact mechanism of these reactions has been the subject of many theories and yet even today is not known with certainty, although it is believed to be a combination of oxidation and polymerization. Consequently owing to the development of serious engine troubles when motor fuels are used which contain or develop very large amounts of gum, for example due to sticking of rings, valves, and other moving parts of the engine and due to clogging up of the intake manifold, etc., motor fuels containing diolefines have not been used with any success.

It has now been found, however, and is the primary object of the present invention, that the advantages of the high anti-detonation blending properties of the diolefines can be used without having the disadvantages of the tendency to form gum. This is accomplished by the use of diolefines in purified form along with materials known as gum inhibitors. Such materials have been used heretofore but not in a fuel to which purified diolefines have been added. Such gum inhibitors have been used to stabilize cracked gasoline against gum formation, and in spite of the fact that it is known that cracked gasoline may contain some diolefines (although the majority of these diolefines and any other even more reactive compounds, if any are present, are generally removed by a suitable treating step such as acid treating, clay treating, etc.), yet it has never been suspected that substantial amounts of purified diolefines themselves could be actually added to a motor fuel, whether derived from a virgin stock, or a cracked stock from which undesirable highly unsaturated compounds have been removed, and yet prevent the formation of

harmful amounts of gum. For example, two commercial gasolines, A and B, purchased on the open market and believed to be largely made from vapor phase cracked gasoline stocks, were analyzed and found to contain only 1.1% and 0.6% diolefines by weight respectively, thus showing that even if large amounts of diolefines had been produced by the cracking operation, they had been substantially all removed before marketing.

In carrying out the present invention, various types of diolefines may be used, for example, butadiene, isoprene, allene, pentadiene, cyclopentadiene, hexadiene, and other conjugated and unconjugated cyclic and straight chain diolefines and they may be added in amounts ranging, for example, from about 3 to 20% or preferably between the limits of about 5 and 10% by volume.

Various types of gum inhibitors including various hydroxy and/or amino derivatives of mono- or poly-nuclear aromatic hydrocarbons or alkylated derivatives thereof may be used, for example, monobenzyl-p-amino phenol, tricresol, amyl-p-amino phenol, alpha-naphthol, alpha-naphthylamine, etc., and they may be used in various amounts between the approximate limits of 1 and 20 mg. per hundred ccs. of fuel, depending upon the nature and quantity of the diolefines added, as well as the type of gasoline base stock used in preparing the blend, although ordinarily the amount to be used will be between the approximate limits of 5 and 15 mg. per hundred ccs. of fuel.

As illustrative of the invention, the following examples are given:

*Example 1*

Butadiene was added to 65 octane number motor fuel in quantity sufficient to make a 5% blend; 10 mg. of monobenzyl-p-amino phenol was added for each one hundred cc. of fuel. The resulting blend had an octane number of 72.3, a breakdown time of 16 hours (2# drop at 100° C.) and a copper dish gum of 3.1 mg./100 cc.

*Example 2*

Isoprene was added to a 73.9 octane number motor fuel in quantity sufficient to make a 5% blend; 10 mg. of monobenzyl-p-amino phenol was added for each 100 cc. of fuel. The resulting blend had an octane number of 76.8, a breakdown time of 16 hours and a copper dish gum of 14.0 mg./100 cc.

In preparing blends according to the present invention other addition agents may be used, for

example, metallo-organic anti-knock agents, particularly those of the lead alkyl type, e. g. 0.5-6.0 cc. per gallon of fuel, of lead tetraethyl, lead tetramethyl, tin tetraethyl and bismuth trimethyl.

The following experimental data will further illustrate methods of carrying out the invention and advantages obtained by the invention.

Table I

| No. | Fuel                            | C. D. gum | Break-down |
|-----|---------------------------------|-----------|------------|
| 1   | Gasoline                        | 3.0       | 11.5       |
| 2   | 5% isoprene in (1)              | 6.0       | 2.5        |
| 3   | 0.5 mg. B. A. P./100 cc. of (2) | 8.0       | 2.7        |
| 4   | 10 mg. B. A. P./100 cc. of (2)  | 11.0      | 10.5       |
| 5   | 20 mg. B. A. P./100 cc. of (2)  | 16.0      | 12+        |
| 6   | 15% isoprene in (1)             | 6.0       | 0.8        |
| 7   | 0.5 mg. B. A. P./100 cc. of (6) | 9.0       | 0.8        |
| 8   | 10 mg. B. A. P./100 cc. of (6)  | 10.0      | 5.1        |
| 9   | 20 mg. B. A. P./100 cc. of (6)  | 15.0      | 4.0        |

\*Benzyl para-amino phenol.

Table II

| No. | Fuel                                     | O. N. C. F. R. |                 | Blending O. N. |                 |
|-----|------------------------------------------|----------------|-----------------|----------------|-----------------|
|     |                                          | No lead        | 3 cc. lead/gal. | No lead        | 3 cc. lead/gal. |
| 10  | Gasoline                                 | 64.5           | 81.1            |                |                 |
| 11  | 10 mg. B. A. P. and 5% isoprene in (10)  | 69.7           | 83.5            | 168.5          | 120.1           |
| 12  | 10 mg. B. A. P. and 15% isoprene in (10) | 73.8           | 84.3            | 126.5          | 102.4           |

The above Tables I and II show that 10 mg. of inhibitor/100 cc. of gasoline were more than sufficient to produce an isoprene-containing blend of satisfactory copper dish gum and breakdown test as well as satisfactory octane number blending characteristics and good lead susceptibility.

Table IIIa

| No. | 5% diolefine | 10 mg./100 cc. inhibitor | Storage | C. D. gum, mg./100 c.c. |         |         |         |
|-----|--------------|--------------------------|---------|-------------------------|---------|---------|---------|
|     |              |                          |         | 0 days                  | 20 days | 56 days | 93 days |
| 13  | None         | None                     | Light   |                         | 3.5     | 5.5     | 4.1     |
| 14  | do           | do                       | Dark    | 4.4                     | 4.3     | 5.0     | 20.3    |
| 15  | Butadiene    | do                       | Light   | 6.9                     | 7.4     | 7.4     | 31.5    |
| 16  | do           | do                       | Dark    |                         | 18.6    | 20.0    | 16.7    |
| 17  | do           | B. A. P.                 | Light   | 17.4                    | 16.4    | 19.7    | 17.4    |
| 18  | do           | do                       | Dark    |                         | 8.2     | 8.3     | 12.1    |
| 19  | do           | T. C.                    | Light   | 8.3                     | 8.6     | 9.8     | 8.2     |
| 20  | do           | do                       | Dark    |                         |         |         |         |

Table IIIb

| No. | 5% diolefine | 10 mg./100 cc. inhibitor | Storage | Breakdown, hours for 2# drop |         |         |         |
|-----|--------------|--------------------------|---------|------------------------------|---------|---------|---------|
|     |              |                          |         | 0 days                       | 20 days | 56 days | 93 days |
| 13  | None         | None                     | Light   |                              | 15      | —       | 10.     |
| 14  | do           | do                       | Dark    | 9.8                          | 10      | 2.0     | 12+ 2.3 |
| 15  | Butadiene    | do                       | Light   | 2.1                          | 2.6     | 2.6     | 2.9 7.5 |
| 16  | do           | do                       | Dark    | 15+                          | 6.9     | 13.0    | 14+ 5.2 |
| 17  | do           | B. A. P.                 | Light   |                              | 16+     | 14.0    | 14.1    |
| 18  | do           | do                       | Dark    | 15+                          | 16+     | 8.8     | 12+     |
| 19  | do           | T. C.                    | Light   |                              |         |         |         |
| 20  | do           | do                       | Dark    |                              |         |         |         |

The above Tables IIIa and IIIb show the copper dish gum and 2# pressure drop or breakdown tests on samples of a refined gasoline alone and with 5% of butadiene with and without 10 mg. of either benzyl para-amino phenol or tricresol per 100 ccs. of fuel, when tested immediately as well as over storage during 20, 56 and 93 days.

The tests in Table IIIa show that the addition of 5% of butadiene to the gasoline (which was a refined aviation gasoline obtained from a Pecos

70 crude base stock) raises the copper dish gum from 4.4 to 6.9 mg. when tested immediately and from 4.1 to 31.5 mg. after 93 days storage in the light. It also shows that the addition of either of the inhibitors (benzyl para-amino phenol or tricresol) resulted in a substantial stabilization of the blended fuel even when stored in light for 93 days (the copper dish gum being 16.7 for the benzyl para-amino phenol inhibitor and 12.1 for the tricresol as compared to 31.5 for the blend without any inhibitor). In tests 17 and 18, the copper dish gum values are higher than in the other tests because the benzyl para-amino phenol is so non-volatile that it remains as a residue and therefore raises the copper dish gum value by an amount practically equal to the weight of the inhibitor used.

From a few additional tests on sludging, it appears that in a fuel to which butadiene has been added, tricresol is unexpectedly superior to benzyl para-amino phenol because for some unknown reason the tricresol has a superior sludge-preventing property in such a blend.

Table IIIb shows that the addition of 5% of butadiene to the plain gasoline base stock lowers the breakdown (a 2# drop from the original 100# of oxygen pressure) from about 10 to 2.1 hours but the addition of 10 mg. of benzyl para-amino phenol or the same amount of tricresol raises 30 the breakdown time to more than 15 hours in each case.

It is understood of course that other known addition agents may be used in preparing motor fuels according to the present invention; for instance, dyes may be added as well as anti-knock agents of other types. Also solvent oils or gum fluxes such as described in the Sloane and Wasson Patent 2,066,234 may be added, and these are particularly useful in a fuel in which substantial

amounts of a relatively non-volatile gum inhibitor such as benzyl para-amino phenol are used.

In carrying out the present invention, it is desirable to prepare a gasoline base stock with less than 2% of hydrocarbons having more aliphatic unsaturation than olefines. In other words, it is desirable to refine either a virgin or cracked gasoline base stock in such a way as by acid treating, clay treating, treating with aluminum chloride, boron fluoride, or other known treating

agents, to produce a gasoline base stock containing less than 2% of diolefines, acetylenes, triolefines, and other highly unsaturated hydrocarbon compounds. If the sulfur content of the resulting base stock is not already low (either by reason of low sulfur crude having been used or by reason of sulfur removal by any of the treatments used for removing the highly unsaturated compounds), suitable additional treatment should be given to reduce the sulfur content down to not more than 0.1% and preferably still lower, to not more than 0.01%. The reduction of the sulfur content is highly desirable not only for the obvious reason of reducing the corrosive tendency of the fuel but also for the even more important purpose of improving the lead susceptibility because it has been found that the diolefines of the present invention have better lead susceptibility than mono-olefines.

The invention is especially valuable in making use of low octane number gasoline base stocks, for instance, those having an octane number less than 65, and is especially useful in straight run fuels. It can of course be applied to high octane number base stocks, e. g. those having an octane number as high as 75 or higher, although in the latter type of fuels the blending octane number of the diolefines is relatively not as high as in the lower octane number fuels.

It is thus seen that whereas in the usual refining practice used heretofore in the preparation of gasoline motor fuels the refining treatment used to reduce the sulfur content, to reduce corrosion and improve lead susceptibility, usually also reduces the content of diolefines and other highly unsaturated compounds, whereby the valuable octane-improving and lead susceptibility characteristics of any diolefines which might have been present would be totally lost, the present invention provides a novel and unexpected method of making use of the said valuable characteristics of the diolefines by adding them in purified form to a suitably purified gasoline base stock. If desired, a gasoline base stock such as one obtained by vapor phase cracking of gas oil

10 or other high-boiling hydrocarbons, or any other suitable hydrocarbon fraction rich in diolefines having from 4 to 10 carbon atoms, can be refined from in a purified condition. For instance, such a crude diolefine-containing fraction may be treated with one or more selective solvent extraction steps, if desired, with successive treatments with sulfuric acid of successively increasing concentrations, in order to obtain a fraction consisting essentially of diolefines which may in turn, if desired, be still further purified before being used as motor fuel blending agents according to the purview of the present invention.

15 The invention is not to be limited to the specific embodiments shown or the specific examples given, nor to any theories advanced as to the operation of the invention, but in the appended claims it is intended to claim all inherent novelty in the invention as broadly as the prior art permits.

We claim:

20 1. A motor fuel consisting essentially of a cracked gasoline which has been substantially freed of unsaturated aliphatic hydrocarbons having more than one double bond per molecule, and which has been reduced to a sulfur content of less than 0.1%, said motor fuel also containing about 5 to 20% of butadiene, about 0.5 to 20 mg. 25 of tricresol per 100 ccs. of fuel, and about 0.5 to 6.0 ccs. of lead tetraethyl per gallon of fuel.

25 2. The method of preparing a motor fuel of improved anti-knock value, high lead susceptibility, and satisfactory stability, which comprises 30 refining a cracked gasoline base stock to substantially free the gasoline of unsaturated aliphatic hydrocarbons containing more than one double bond per molecule and to reduce the sulfur content of the gasoline to less than 0.1%, adding to 35 the thus refined cracked gasoline pure butadiene in an amount of about 5% to 10% by volume, and a small amount of gum inhibiting phenolic compound.

40 GEORGE H. FREYERMUTH.  
ANTHONY E. ROBERTSON.